

Jan. 26, 1971

TSUTOMU HAMAOKA ET AL  
COLOR PHOTOGRAPHIC SILVER HALIDE EMULSION  
CONTAINING MAGENTA COUPLERS

Filed July 12, 1967

3,558,319



INVENTORS

TSUTOMU HAMAOKA  
KAZUYA SANO  
MAKOTO YOSHIDA  
YASUSHI OISHI  
TAKESHI HIROSE

Aughron, Rotwell, mis, Zinn & maggent  
ATTORNEYS



stituent being chosen from the class consisting of halogens, lower alkyl groups and lower alkoxy groups.

The RCO group contributes the solubility of the coupler as well as its resistance to diffusion. If the RCO group carries less than 18 carbon atoms, the coupler wanders out of the layer because of the low solubility in the organic solvent and low diffusion-resistance, resulting in a worsened color reproduction. On the other hand, an excessively large RCO group, having more than 25 carbon atoms, brings about an excessively large molecular weight and thus too small an extinction per volume. Moreover the dispersion force due to this part of the molecule reduces the solubility of the coupler. The RCO group is most suitably located meta to the ureido group since the compound of this location provides a higher solubility than its isomers. For example, the para isomer gives the dye of the absorption characteristics as excellent as the meta isomer but cannot be employed owing to its low solubility. This feature is well illustrated in Table 1.

The RCO group is preferably a substituted or an unsubstituted aliphatic acyl group or one of the following:



wherein  $\text{R}_1$  represents a hydrogen atom or an alkyl group having not more than 3 carbon atoms,  $\text{R}_2$  represents an alkyl group having not more than 5 carbon atoms,  $\text{R}_3$  represents an alkyl group having from 5 to 16 carbon atoms, and  $n$  is an integer from 1 to 5.

The ortho substituent of the Ar group is quite important because the lack of the substituent gives rise to too low a solubility, and an excessive coupling activity, which leads to fogging, and thus, to worsening of the image quality.

The effect of the ortho substituent is believed to be due to loss of the co-planarity of the pyrazolone and the aryl nuclei, which are affected by many kinds of substituents, such as halogens, alkyl groups and alkoxy groups. These substituents are also effective in preventing the yellowing of the couplers by light. In particular, those that carry two substituents at the ortho positions are remarkably resistant to the action of light.

#### BRIEF DESCRIPTION OF THE DRAWING

FIGS. 1, 2 and 3 show the spectral absorption curves of dye images obtained by processing couplers I, IV and IX with 2-amino-5-diethylaminotoluene compared with those from the corresponding reference couplers. Curves *a* and *b* of FIG. 1, *c* and *d* of FIG. 2 and *e* and *f* of FIG. 3 correspond to couplers I, A, IV, B, IX and H, respectively.

#### DETAILED DESCRIPTION OF THE INVENTION

The couplers suitably used in the present invention are exemplified by the following:

(I)





30 Each of the following compounds has something in common with couplers I-XIII. Comparison of the two groups will serve to illustrate the merits of the couplers of the present invention.



(D)



(E)



(F)



(G)



(H)



(J)



(K)



8

15 The magenta color image obtained from the color photographic material containing the coupler of this invention fades only reluctantly by the action of light, heat and environmental humidity, as is shown in Example 4, and the remaining coupler scarcely yellows when exposed to strong radiation. This makes this invention especially valuable from the viewpoint of image preservation.

20 In the second place, the coupler of this invention gives high sensitivity and desirable gradation to the photographic emulsion, while giving rise to little fogging owing to its moderate coupling activity. In addition, the present 25 coupler shows a high rate of conversion to azomethine dyes and thus increases the sensitivity even more. This results in a smaller amount of coupler needed, and thus, in a thinner emulsion layer, which improves the image quality and the rate of development.

30 Thirdly, the coupler of this invention has a high solubility in such organic solvents as di-n-butyl phthalate and ethyl acetate. In other words, only a small amount of solvent is needed to disperse this kind of coupler. This necessarily simplifies the production of the photographic material. It also excludes the need for a thick layer, guaranteeing higher quality of the image, a higher development rate, and better mechanical properties of the emulsion layer. Table 1 shows the solubilities and melting points of 35 couplers I, V, IX and X, together with those of reference couplers C, D, F and B, which have structures similar to couplers I, V, IX and X, respectively. The solubility has been designated as the amount of ethyl acetate needed to dissolve 1 part of the coupler at 60° C. It should be noted that a smaller value corresponds to a higher solubility.

TABLE I.—MELTING POINTS AND SOLUBILITIES OF THE COUPLERS OF THIS INVENTION COMPARED WITH THE REFERENCE COUPLERS

| Coupler                         | Coupler of this invention |     |     |     | Reference coupler |     |     |     |
|---------------------------------|---------------------------|-----|-----|-----|-------------------|-----|-----|-----|
|                                 | I                         | V   | IX  | X   | C                 | D   | F   | B   |
| Melting point.....              | 182                       | 156 | 150 | 139 | 204               | 220 | 224 | 120 |
| Solubility (defined above)..... | 2.5                       | 2.0 | 1.5 | 1.0 | 7.5               | 7.5 | 7.5 | 2.0 |

60 In the fourth place, dyes from the couplers of this invention give absorption characteristics suited for the subtractive color process.

65 Referring to the drawing, all the figures indicate that the couplers of the present invention, which carry 3-(4-acylaminophenyl-ureido) substituents are superior to the reference couplers of known types, which carry 3-acylaminoo substituents, especially with regard to the absorption in the shorter wave-length region.

70 Such excellent absorption characteristics are believed to be due not only to the high solubility of the dyes in the co-existing solvent, but also to their own nature.

75 Table 2 illustrates the absorption characteristics of ethyl acetate of dyes obtained by the oxidative coupling of the couplers of this invention with 2-amino-5-N,N-diethylaminotoluene along with those from the corresponding reference couplers.

TABLE 2.—ABSORPTION CHARACTERISTICS OF DYES IN ETHYL ACETATE

|                                                  | Coupers of the invention |      | Reference coupers |      |      |      |      |      |
|--------------------------------------------------|--------------------------|------|-------------------|------|------|------|------|------|
|                                                  | I                        | V    | A                 | B    | E    | G    | J    | K    |
| Primary absorption max. wave length (m $\mu$ )   | 534                      | 541  | 525               | 535  | 537  | 519  | 541  | 539  |
| Secondary absorption max. wave length (m $\mu$ ) | 438                      | 431  | 441               | 438  | 435  | 445  | 431  | 438  |
| B-value                                          | 0.14                     | 0.13 | 0.21              | 0.17 | 0.16 | 0.46 | 0.17 | 0.17 |
| W-value (m $\mu$ )                               | 74                       | 76   | 79                | 78   | 75   | 78   | 79   | 80   |
| S-value                                          | 0.21                     | 0.19 | 0.26              | 0.22 | 0.29 | 0.35 | 0.24 | 0.24 |

It will be clearly seen that the coupers of the present invention are especially suited for color photography because of unusually small B-(second absorption) and S-(red absorption) values while maintaining moderate W-values.

The following exemplify the preparation of these compounds:

#### Preparation of Compound I

(a) Preparation of m-nitrophenyl isocyanate.—In a 5-liter three-necked flask were placed 500 ml. of ethyl acetate, saturated with phosgene at room temperature. While refluxing and passing phosgene, 150 g. of m-nitroaniline, dissolved in 1.5 liters of dry ethyl acetate were gradually added. After addition of m-nitroaniline over 4 hours at such a rate as to avoid accumulation of nitroniline hydrochloride, phosgene was passed in for 5 minutes more, ethyl acetate was distilled out, and the viscous residue was distilled under reduced pressure by means of an aspirator. One hundred and thirty grams of m-nitrophenyl isocyanate boiling at 161° C./25 mm. Hg was obtained.

(b) Synthesis of 1-(2-chlorophenyl)-3-(3-nitrophenylureido) - 5-pyrazolone.—In a 1 liter three-necked flask were placed 76 g. of 1-(2-chlorophenyl)-3 - amino-5-pyrazolone (J. Am. Chem. Soc., 66 1862 (1944)) and 600 ml. of acetonitrile. While stirring under reflux, a solution consisting of 200 ml. of acetonitrile and 60 g. of m-nitrophenyl isocyanate was added dropwise into the system. During the addition, the pyrazolone went into solution then the solution rapidly began to separate crystals. After stirring for 2 hours under reflux, the product was collected by filtration and was recrystallized from a mixture of one part of dimethylformamide and two parts of ethanol to give 50 g. of the compound melting at 254° C.

(c) Reduction of the nitro group.—While stirring under reflux the whole amount of the nitro compound obtained above in 500 ml. of methanol, 500 ml. of glacial acetic acid and 50 ml. of water, 50 g. of reduced iron powder were added gradually. After 2 hours, the reaction mixture was poured into 5 liters of hot water and was allowed to stand overnight. The product was collected by filtration and recrystallized from a solvent mixture of ethanol and acetonitrile (1:1) to give 30 g. of the amine melting at 207° C.

(d) Synthesis of Compound I.—A mixture of 15 g. of the amine obtained in step (c), 4.5 g. of sodium acetate and 260 ml. of glacial acetic acid was warmed to 50–60° C., while stirring and into the solution was gradually added a solution of 14.5 g. of 2,4-di-t-amylphenoxyacetyl chloride in 75 ml. of glacial acetic acid. The mixture was allowed to react for 2 hours at this temperature.

The reaction mixture was poured into 1.5 liters of cold water and the product was collected by filtration, dried and recrystallized from a mixture of methanol and acetonitrile (1:1) to give 8 g. of Compound I melting at 182° C.

#### Preparation of Compound II

A mixture of 15 g. of the amine obtained in step (c) in the preparation of Compound I, 4.5 of sodium acetate and 260 ml. of glacial acetic acid was warmed to 50–60° C. While stirring, a solution of 14.5 g. of 2,4-di-sec-amylphenoxyacetyl chloride in 75 ml. of glacial acetic acid was added dropwise. The mixture was allowed to react for 2 more hours at this temperature.

The reaction mixture was poured into 1.5 liters of cold water and the product was collected by filtration, dried and recrystallized from a mixture of acetone and methanol (1:1) to give 6 g. of Compound II melting at 174° C.

#### Preparation of Compound IV

(a) Synthesis of 1-(2,4,6-trichlorophenyl)-3-(3-nitrophenylureido)-5-pyrazolone.—In a 1-liter three-necked flask were placed 84 g. of 1-(2,4,6-trichlorophenyl)-3-amino-5-pyrazolone (see U.S. Pat. 2,600,788) and 600 ml. of anhydrous acetonitrile. While stirring under reflux, a solution consisting of 200 ml. of anhydrous acetonitrile and 49 g. of m-nitrophenyl isocyanate was added gradually. After the addition, the mixture became clear and after about 30 minutes began to separate a large amount of crystals which were collected by filtration and washed with hot acetonitrile to give 40 g. of the nitro compound melting at 232° C.

(b) Reduction of the nitro compound.—The reduction of the nitro compound was conducted in the same way as the preparation of Compound I. Thus, by reduction of 40 g. of the nitro compound obtained above, 15 g. of the amine melting at 224° C. was obtained.

(c) Synthesis of Compound IV.—In 240 ml. of glacial acetic acid were suspended 15 g. of the amine obtained above, and 4.5 g. of sodium acetate, and, while stirring at 50–50° C., a solution of 13 g. of 2,4-di-t-amylphenoxyacetyl chloride and 80 ml. of glacial acetic acid were gradually added dropwise into the suspension. After the addition, the mixture was allowed to react for 2 more hours. The reaction mixture was poured into 1.5 liters of cold water. The product was collected and was recrystallized, after drying, from a solvent mixture of acetonitrile and methanol (1:1) to give 9 g. of Compound IV melting at 198° C.

#### Preparation of Compound VI

(a) Preparation of 1-(2-ethoxyphenyl) - 3 - amino-5-pyrazoline.—A mixture of 64 g. of o-ethoxyphenylhydrazine, 360 ml. of methanol and 70 g. of anhydrous sodium acetate was cooled below 10° C., and 90 g. of ethyl  $\beta$ -ethoxy- $\beta$ -iminopropionate hydrochloride were gradually added. The resulting solution was stirred for 90 minutes at room temperature.

Then, a sodium methylate solution prepared from 42 g. of sodium metal and 600 ml. of methanol maintained at 10° C. was added to the system. The solution was stirred for 90 more minutes at room temperature. Then, the reaction mixture was poured into 3 liters of cold water. After neutralization with acetic acid, the product was extracted with ethyl acetate and dried over anhydrous sodium sulfate. The solvent was removed under reduced pressure and the remaining syrup was washed with hexane and digested with ether until it crystallized. It was recrystallized from ethyl acetate to give 64 g. of the pyrazolone melting at 166° C.

(b) Preparation of 1 - (2 - ethoxyphenyl)-3-(3-nitrophenylureido)-5-pyrazolone.—By the reaction of 44 g. of the pyrazolone prepared above with 33 g. of m-nitrophenyl isocyanate in the same procedure as step (b) of the preparation of Compound I, 30 g. of the above compound melting at 210° C. was obtained.

(c) Reduction of the nitro group.—The whole amount of the nitro compound prepared by step (b) was re-

## 11

duced as in step (c) of the preparation of Compound I. The product thus obtained was recrystallized from a solvent mixture of acetonitrile and ethanol (1:1) containing a small amount of methyl Cellosolve to give 7.2 g. of the amine melting at 190° C.

(d) Synthesis of Compound VI.—7.2 g. of the amine prepared above and 2 g. of anhydrous sodium acetate were suspended in 100 ml. of glacial acetic acid and, while stirring, an acetic acid solution of 6.4 g. of 2,4-di-t-aminophenoxyacetyl chloride was added dropwise into the suspension. After 2 hours, the reaction mixture was poured into cold water. The product was collected by filtration, washed well with water and dried to give 7 g. of Compound VI melting at 120° C.

## Preparation of Compound IX

(a) Preparation of 1-(2,6-dichloro-4-methylphenyl)-3-(3-nitrophenylureido)-5-pyrazolone.—In 700 ml. of acetonitrile were dissolved 100 g. of 1-(2,6-dichloro-4-methylphenyl)-3-amino-5-pyrazolone and while stirring under reflux, 64 g. of m-nitrophenyl isocyanate dissolved in 200 ml. of acetonitrile were added dropwise. After about 40 minutes a large quantity of product precipitated. After 1.5 hours, the precipitates were collected by filtration and washed with hot acetonitrile to give 110 g. of the nitro compound melting at 248° C.

The aminopyrazolone used here had been prepared by the reaction of 2,6-dichloro-4-methylphenylhydrazine with ethyl  $\beta$ -amino- $\beta$ -ethoxy-propionate in a similar way as step (a) of the preparation of Compound VI followed by recrystallization of the product from acetonitrile.

(b) Reduction of the nitro compound.—In the mixture of 500 ml. of methanol, 500 ml. of glacial acetic acid and 50 ml. of water were suspended 50 g. of the nitro compound obtained in step (a) and reduced with iron powder according to step (c) of the preparation of Compound I. The product was recrystallized from the mixture of 2 parts of methanol and 1 part of acetonitrile to give 23 g. of the amino compound melting at 225° C.

(c) Synthesis of Compound IX.—In 360 g. of glacial acetic acid were placed 23 g. of the amine thus prepared and 6 g. of anhydrous sodium acetate. A solution of 19.5 g. of 2,4-di-t-aminophenoxyacetyl chloride in 72 ml. of glacial acetic acid was added dropwise into the solution within 10 minutes. After 2 hours, the mixture was poured into cold water to precipitate the product, which was recrystallized from a mixture of 3 parts of methanol and 2 parts of acetonitrile to give 10 g. of Compound IX melting at 150° C.

## Preparation of Compound X

(a) Preparation of 1-(2,6-dichloro-4-methoxyphenyl)-3-(3-nitro-phenylureido)-5-pyrazolone.—In 500 ml. of acetonitrile were treated 40 g. of m-nitrophenyl isocyanate with 67 g. of 1-(2,6-dichloro-4-methoxyphenyl)-3-amino-5-pyrazolone, (see British Pat. 904,852) according to step (b) of the preparation of Compound I to give 67 g. of the nitro compound melting at 227° C.

(b) Reduction of the nitro group.—In a mixture of 670 ml. of methanol, 670 ml. of glacial acetic acid and 67 ml. of water were reduced 67 g. of the nitro compound obtained above by means of 67 g. of reduced iron powder, and the product thus prepared was recrystallized from a mixture of 3 parts of ethanol and 2 parts of dimethylformamide to provide 52 g. of the amine, melting at 200-201° C.

(c) Synthesis of Compound X.—In 520 ml. of glacial acetic acid were suspended 52 g. of the amino compound prepared in step (b) and 12.5 g. of anhydrous sodium acetate, and while stirring, 40 g. of 2,4-di-t-aminophenoxyacetyl chloride and 120 ml. of glacial acetic acid were added dropwise into the suspension at 50-60° C. After 1 hour, the mixture was poured into cold water to precipitate the product, which was collected by filtration, dried,

## 12

and recrystallized from methanol to give 69 g. of the crystal of Compound X melting at 139° C.

Preparation of Compound XIII.—In 200 ml. of glacial acetic acid were suspended 10 g. of the amine prepared by step (c) of the preparation of Compound I and 2.5 g. of anhydrous sodium acetate and, while stirring at 50-60° C., a solution of 8 g. of palmitoyl chloride in 50 ml. of glacial acetic acid was added dropwise into the suspension within 5 minutes. After 1 hour, the reaction mixture was poured into 1 liter of cold water. The product was collected by filtration, dried and recrystallized twice from a mixture of methanol and acetonitrile (1:1) and once from ethanol to give 4 g. of Compound XIII melting at 178° C. Couplers described in this application can be mixed with a small amount of cyan- or yellow-forming coupler to improve the color reproduction according to Japanese patent publication No. 391/1965.

This invention can be satisfactorily applied to many types of light-sensitive materials, for example, color-printing papers, positive color films, negative color films, reversal color films and so forth.

Also this invention is expected to be applicable not only to so-called multilayer color photographic materials, but also to so-called mixed grain type ones. The invention will further be explained by the following examples.

## EXAMPLE 1

A solution prepared by warming to 70° C. a mixture of 15 g. of Compound I, 30 g. of di-n-butyl phthalate and 20 ml. of butyl acetate was added to 300 ml. of an aqueous solution of 1.0 g. of sodium dodecylbenzenesulfonate and 25 g. of gelatin. The mixture was stirred for 30 minutes in a homogenizer, and the whole amount of the mixture was mixed with 500 g. of a green-sensitive photographic emulsion.

After addition of 30 ml. of a 3% acetone solution of triethylene-phosphoramide and adjustment of the pH to 7.0, the resulting composition was applied to cellulose triacetate film to a dry-thickness of  $5.0 \times 10^{-4}$  cm.

The coating contained  $5.8 \times 10^{-3}$  mole of silver iodobromide and  $7.2 \times 10^{-4}$  mole of the coupler per square meter. The film was exposed and subjected to the following processing steps to yield a clear magenta image with an absorption maximum at 551 m $\mu$ . The spectral absorption curve has been shown in FIG. 1 by curve  $\alpha$ .

## COLOR DEVELOPMENT PROCESSES

| Step                   | Temperature, °C. | Period, minutes |
|------------------------|------------------|-----------------|
| Color development..... | 21               | 10              |
| Rinsing.....           | 21               | 1               |
| First fixing.....      | 21               | 4               |
| Rinsing.....           | 21               | 3               |
| Bleaching.....         | 21               | 3               |
| Rinsing.....           | 21               | 2               |
| Second fixing.....     | 21               | 3               |
| Washing.....           | 18               | 20              |

The compositions used in the above processes are as follows:

Color developer (a) (pH 10.5):  
Water—1,000 ml.  
2-amino-5-diethylaminotoluene hydrochloride—2.5 g.  
Sodium sulfite (anhydrous)—10 g.  
Sodium carbonate, monohydrate—47 g.  
Potassium bromide—2 g.

## Fixing solution (pH 4.5):

Water—1,000 ml.  
Sodium thiosulfate 6H<sub>2</sub>O—80 g.

Sodium sulfite—5 g.

Borax—6 g.

Glacial acetic acid—4 ml.

Potassium alum—7 g.

## Bleaching solution (pH 7.2):

Water—1,000 ml.

Potassium ferricyanide—17 g.

Boric acid—10 g.  
Borax—5 g.  
Potassium bromide—7 g.

## EXAMPLE 2

A solution prepared by warming to 70° C. a mixture of 10 g. of Compound X, 30 g. of tricresyl phosphate, and 10 ml. of ethyl acetate was added to 100 ml. of an aqueous solution containing 0.5 g. of sodium dodecyl sulfate and 7 g. of gelatin at 60° C., and the resulting mixture was stirred vigorously by means of an homogenizer to disperse the coupler finely together with the solvent.

The whole amount of the emulsion thus obtained was added to 540 g. of a green-sensitive photographic emulsion. After addition of 30 ml. of 3% acetone solution of triethylenephosphoramide as a hardening agent and 7 g. of polyvinyl pyrrolidone, the resulting composition was applied to baryta paper as the middle layer to a dry-thickness of  $4 \times 10^{-4}$  cm. Its bottom layer was a blue-sensitive photographic emulsion layer containing an emulsified dispersion of coupler (L) having the following structure. On the middle layer thus formed was coated as the top layer a red-sensitive emulsion containing an emulsified dispersion of coupler (M) shown below.



In this case the middle layer contained  $3.6 \times 10^{-4}$  mol coupler and  $2.9 \times 10^{-3}$  mol silver chlorobromide per square meter. The completed color printing paper was exposed to graduated intensities of green light and developed as in Example 1. The magenta image thus obtained satisfied the requirements of color printing paper. Further, when this paper was exposed through a negative color film and developed as mentioned above, clear-color images were obtained.

## EXAMPLE 3

A mixture of 6 g. of Compound IX and 18 g. of dibutyl phthalate was warmed to 80° C., and added to 50 ml. of an aqueous solution containing 5 g. of gelatin and 0.3 g. of sodium dodecylbenzenesulfonate, and the resulting mixture was stirred vigorously by means of an homogenizer to prepare an emulsified dispersion.

The whole amount of the coupler-containing emulsified dispersion was mixed with 200 g. of a photographic emulsion. After addition of 10 ml. of a 3% acetone solution of triethylene phosphoramide as a hardening agent, the mixture was applied to a cellulose triacetate film to a dry-thickness of  $6 \times 10^{-4}$  cm. and dried. In this case, the coating contained  $7.2 \times 10^{-4}$  mol coupler and  $5.8 \times 10^{-3}$  mol silver iodobromide per square meter. The film was exposed to graduated intensities of light with aid of a sensitometer and developed for 6 minutes at 24° C. in a developer of the following composition and then washed with water for 15 minutes at the same temperature; then it was exposed uniformly to white light and color-developed as described in Example 1.

Black and white developer (pH 10.8):

Water—1,000 ml.

Metol—3 g.

Sodium sulfite (anhydrous)—50 g.

Sodium carbonate, monohydrate—100 g.

Potassium thiocyanate—3.6 g.

Potassium bromide—2 g.

The reversal magenta color image thus obtained had an absorption maximum at 554 m $\mu$ . The spectral absorption curve has been shown in FIG. 3 of the attached drawing as curve e.

## EXAMPLE 4

Two films (P) and (Q) were prepared as follows:

Film (P).—A solution prepared by heating to 70° C. a mixture of 15 g. of Compound IV, 30 g. of tricresyl phosphate and 20 ml. of butyl acetate was mixed with 300 ml. of an aqueous solution containing 25 g. of gelatin and 1.0 g. of sodium dodecylbenzenesulfonate. The mixture was stirred for 30 minutes by means of a homoblender to disperse the coupler. The whole amount of the dispersion was mixed with 500 g. of photographic emulsion. After addition of 30 ml. of 3% acetone solution of triethylenephosphoramide as a hardening agent, the mixture was neutralized to pH 7.0 and was applied to a cellulose triacetate film to a dry-thickness of  $5.0 \times 10^{-4}$  cm. The coating contained  $7.2 \times 10^{-4}$  mol coupler and  $5.8 \times 10^{-3}$  mol silver iodobromide per square meter.

Film (Q).—A similar procedure to the preparation of Film (P) was repeated using Compound B (control) instead of Compound IV.

The films were exposed to graduated intensities of light by means of a sensitometer and processed in the same manner as Example 1. Their photographic properties are as follows:

| Sample | Coupler | Sensitivity (relative) |     | Gamma | Maximum density |
|--------|---------|------------------------|-----|-------|-----------------|
|        |         | Fog                    | 120 |       |                 |
| Film P | IV      | 0.09                   | 120 | 2.20  | 3.05            |
| Film Q | B       | 0.08                   | 100 | 1.61  | 2.16            |

The fastness of the color image was tested, and the results are shown in the following table:

| Sample | Coupler | (A), initial density |     | (B), initial increase in blue density |     | (C), initial density |     | (D), initial density |     |
|--------|---------|----------------------|-----|---------------------------------------|-----|----------------------|-----|----------------------|-----|
|        |         | 2.0                  | 1.0 | 2.0                                   | 1.0 | 2.0                  | 1.0 | 2.0                  | 1.0 |
| Film P | IV      | 20                   | 30  | 0.03                                  | 5   | 7                    | 13  | 22                   |     |
| Film Q | B       | 49                   | 52  | 0.04                                  | 11  | 15                   | 46  | 58                   |     |

NOTE: (A) Fading (percent) by light (after 40 hours, exposure in a xenon tester), (B) Coloring of uncoupled portion by light (after 40 hours, exposure in a xenon tester), (C) Fading (percent) at a high temperature and a high humidity (60° C. 75% RH for 20 days), and (D) Fading (percent) by heat (at 120° C., for 4 hours).

From the above results, it is clear that Film (P), (Coupler IV) according to the present invention, gives a high sensitivity, a high gamma and a high maximum density compared with those of Film Q containing the conventional coupler (B), and that the color image obtained is markedly fast to light, heat and humidity. Moreover, even intense radiation did not cause yellowing due to the remaining coupler.

The spectral absorption curve of the color image formed by Compound IV has been shown in FIG. 2 of the attached drawing by curve c.

What is claimed is:

1. A color photographic silver halide emulsion containing at least one magenta coupler of the formula



wherein RCO represents an acyl group having from 18 to 25 carbon atoms and Ar represents a phenyl group having at least one substituent at the ortho position, the substituent being one selected from the group consisting of halogens, alkyl groups and alkoxy groups.

2. A color photographic silver halide emulsion as defined in claim 1 where the compound is:



3. A color photographic silver halide emulsion as defined in claim 1 where the compound is:



4. A color photographic silver halide emulsion as defined in claim 1 where the compound is:



5. A color photographic silver halide emulsion as defined in claim 1 where the compound is:



6. A color photographic silver halide emulsion as defined in claim 1 where the compound is:



7. A color photographic silver halide emulsion as defined in claim 1 where the compound is:



8. A color photographic silver halide emulsion as defined in claim 1 where the compound is:



9. A color photographic silver halide emulsion as defined in claim 1 where the compound is:



10. A color photographic silver halide emulsion as defined in claim 1 where the compound is:



17

11. A color photographic silver halide emulsion as defined in claim 1 where the compound is:



18

13. A color photographic silver halide emulsion as defined in claim 1 where the compound is:



14. A color photographic silver halide emulsion as defined in claim 1 where the compound is:



12. A color photographic silver halide emulsion as defined in claim 1 where the compound is:



#### References Cited

#### UNITED STATES PATENTS

3,393,071 7/1968 Monbaliu et al. ----- 96—100  
3,462,270 8/1969 Eynde et al. ----- 96—100

J. TRAVIS BROWN, Primary Examiner

U.S. Cl. X.R.

96—74; 260—310